

# UNITED STATES PATENT OFFICE.

JOSE SANTIAGO VILLACORTA, OF SAN ILDEFONSO, BULACAN, PHILIPPINE ISLANDS.

## PROCESS OF TREATING TOBACCO-LEAF.

1,401,106.

Specification of Letters Patent. Patented Dec. 20, 1921.

No Drawing.

Application filed August 9, 1921. Serial No. 490,975.

To all whom it may concern:

Be it known that I, JOSE S. VILLACORTA, a citizen of the United States, residing at San Ildefonso, Bulacan, Philippine Islands, have invented certain new and useful Improvements in Processes of Treating Tobacco-Leaf; and I do hereby declare the following to be a full, clear, and exact description of the invention, such as will enable others skilled in the art to which it appertains to make and use the same.

My invention relates to improvements in the treatment of tobacco leaf in order to render the ordinary leaf suitable for cigar wrapping purposes, and to do away with the necessity and expense of employing high-priced and specially grown tobacco leaves for wrappers for cigars.

The tobacco leaf to be subjected to the dinitocinizing and bleaching process should be broad, of medium thickness, thoroughly cured, and as free from physical defects as possible, that is, more especially it should not be torn or have holes therein. During the experiments four varieties of tobacco were used, viz: Sumatra wrapper, tirona hybrid, Connecticut broad leaf (raised by the College of Agriculture, University of the Philippines) and Isabela wrapper, all of which have been bought from the Philippine markets. Any tobacco leaf, however, will serve the purpose, provided it is well cured and free from physical defects. The treatment complete comprises two distinct processes, the one mechanical, the other chemical, which will be described as follows:

### 1. Mechanical process.

The leaf so selected is to be divided into halves by cutting it through the midrib starting from the distal down to the proximal end. In order to facilitate the division, the leaf should be moistened with water. The leaf thus divided into halves is pressed between two sheets of paper, in order to remove the excess of moisture.

The next step is to place the leaf on a sheet of abrasive glass paper and pound it lightly with a rubber hammer with soft round head, or roll it with a small heavy roller. This process is necessary in order to produce minute holes or bruises all over the surface, so as to insure a thorough penetra-

tion of water or chemical solutions, thereby shortening as much as possible the time of immersion of the leaf, otherwise it becomes too macerated and unserviceable due to prolonged immersion.

### 2. Chemical process.

The chemical process is conducted in successive steps, which are enumerated below, for the sake of convenience.

*First step.*—The leaves thus divided, pressed and gently bruised are immersed in clean water, preferably distilled water, for twenty-four hours, changing, however, the water at the end of the first ten hours. This is necessary because the nicotin or other soluble substances, if not removed, will interfere with the oxidizing action of the sodium-chlorid-potassium-permanganate solution.

*Second step.*—The leaves are carefully washed in a basin with tap water until the washings run out clear.

*Third step.*—The leaves are then transferred to a solution of sodium-chlorid (one gram of NACL to 1,000 cc. of water, preferably distilled water) containing potassium permanganate in the proportion of 4.5 grams per thousand. Two leaves, *i. e.* four halves should be placed in one liter of such solution and allowed to remain there from one and a half to three hours, depending upon the degree and extent of bleaching which is desired.

After this oxidization, the semi-translucent color of the leaf, after dinitocinization, becomes opaque and dark. This change of color may be used as a guide as to length of exposure to oxidization.

The above mentioned solution may be used three or four times without exhausting its oxidizing properties. This is to economize expense in the use of potassium permanganate.

*Fourth step.*—After the exposure, as described in the next preceding step, the leaves are washed again as described in the second step. After this the leaves are immersed in a 5.5 grams per thousand solution of oxalic acid with 1 cc. of citric acid, or 2 cc. of lemon juice to the liter. Four half leaves should be placed in one liter of such solution from 45 minutes to 2 hours, after which they are to be washed again

as described in the second step. It is of paramount importance that the washings after exposure to the chemical solutions as described in the third and fourth steps should be carried out well, thoroughly and with extreme care in order to insure a complete and absolute freedom from even the minutest trace of any chemical element on the tobacco leaf. During the process of immersion, either in water or chemical solutions, air bubbles should be avoided from being kept under or between the leaves, because the portions of the leaf covered by the bubbles will not be affected by the chemicals.

*Fifth step.*—After this last washing the leaves are hung up for awhile to allow the excess of water to dribble down. After this the leaves are placed between two sheets of paper, such as Chinese paper or the ordinary blotting paper, and pressed down for a period of time sufficient for the absorption of the excess of water by the paper, but the leaves should not be left there until they become dry, otherwise they will be too brittle to be used for the cigar wrapper. In this still damp condition the leaves are ready for cigar wrapper purposes.

The commercial purpose of the process above described is to improve the appearance of the cigars so that they may command a much higher price in the market; and also to do away with the necessity of special tobacco wrappers which are especially raised for the purpose at great expense; because, as above stated, any suitable kind of tobacco leaf may be submitted to the same process with the same result.

As to the taste, cigars wrapped with the dinicotinized and bleached wrapper made by the process hereinbefore described do not differ from cigars wrapped, otherwise, since the fillings are not changed.

It will be obvious that changes might be made in the mode of treatment and the length of treatment, and the proportions of the various ingredients in the chemicals used; and I do not mean to limit the invention to such details except as particularly pointed out in the claims.

Having thus described my invention what

I claim and desire to secure by Letters Patent of the United States is:—

1. A process for the treatment of tobacco which comprises (a) bruising or destroying the continuity of the leaf surface, (b) washing to remove the nicotin and soluble substances, (c) treating with an oxidizing compound, and (d) washing to remove any excess of chemicals. 55 60

2. A process for the treatment of tobacco which comprises (a) bruising or destroying the continuity of the leaf surface, (b) washing to remove the nicotin and soluble substances, (c) treating with a solution of potassium permanganate, (d) neutralizing with a solution of oxalic and citric acids, and (e) washing to remove any excess of chemicals. 65

3. A process for the treatment of tobacco which comprises (a) bruising or destroying the continuity of the leaf surface, (b) washing to remove the nicotin and soluble substances, (c) treating with a solution of potassium permanganate and sodium chlorid, 70 75 (d) neutralizing with a solution of oxalic and citric acids, and (e) washing to remove any excess of chemicals.

4. A process for the treatment of tobacco which comprises (a) bruising or destroying the continuity of the leaf surface, (b) washing to remove the nicotin and soluble substances, (c) treating with a solution of potassium permanganate of approximately 4.5 grams per thousand, (d) neutralizing and 80 85 bleaching with a solution of oxalic and citric acids, and (e) washing to remove any excess of chemicals.

5. A process for the treatment of tobacco which comprises (a) bruising or destroying 90 the continuity of the leaf surfaces, (b) washing to remove the nicotin and soluble substances, (c) treating with a solution of potassium permanganate and sodium chlorid, comprising about 4.5 grams per thousand of permanganate, and about 1 gram per thousand of sodium chlorid, (d) neutralizing and bleaching with a solution of oxalic and citric acids, and (e) washing to remove any excess of chemicals. 95

JOSÉ SANTIAGO VILLACORTA.